

March 1, 1932.

L. L. JONES ET AL

1,847,653

MANUFACTURE OF RESISTANCE UNITS

Filed March 12, 1928

Fig. 1.



Fig. 2.



INVENTOR  
Lester L. Jones  
Joseph A. Flanzer

BY

*Lester L. Jones*  
ATTORNEYS

## UNITED STATES PATENT OFFICE

LESTER L. JONES, OF ORADELL, NEW JERSEY, AND JOSEPH A. FLANZER, OF BROOKLYN, NEW YORK, ASSIGNORS TO TECHNIDYNE CORPORATION, OF NEW YORK, N. Y., A CORPORATION OF NEW YORK

## MANUFACTURE OF RESISTANCE UNITS

Application filed March 12, 1928. Serial No. 260,987.

This invention relates to the art of making resistances, and relates more particularly to the manufacture of resistance units having painted or coated resistance films or strips; and has special reference to the making of resistance elements of this nature having predetermined or desired temperature coefficients.

In the copending application of Lester L. Jones et al., Ser. No. 61,326, filed Oct. 8, 1925, and which issued as Patent 1,762,990, June 10, 1930, there is disclosed the art of making a resistance paint capable of being applied to such insulating substances as glass, porcelain, bakelite and the like and capable of being applied by a coating or painting process to produce resistance units or elements, the coating of resistance material comprising finely divided graphite held in a binder such as an alkaline silicate. These resistance coatings when thus applied form very thin resistance films having a thickness of the order of magnitude of 0.25 thousandths of an inch, which resistance films are produced in continuous and unbroken coatings having a comparatively low specific resistance. In another copending application of Lester L. Jones et al., Ser. No. 167,583, filed Feb. 11, 1927, which issued as Patent 1,773,105, Aug. 19, 1930, there is disclosed an improved resistance paint and method of making the same also embodying a finely divided graphite held in a binder which may be coated or painted on mica, glass and other bases to form thin non-hygrosopic resistance films.

These graphite resistance paints or coatings possess a negative temperature coefficient which becomes pronounced at relatively high operating temperatures; and this may become objectionable, particularly where it is desired to employ the resistance units in circuits where it is necessary to maintain the resistance values constant with a substantial degree of accuracy, as within 1%, and over a large range of operating temperatures, as for example, between room temperature and 200°C. The principal object of our present invention is directed to the making of resistance units or elements, employing these graphite paints or coatings, in which the negative tempera-

ture coefficient may be compensated for or eliminated so that the resistance values of the units may be maintained substantially constant over wide temperature variations, or more broadly in which the temperature coefficient may be fixed at any desired low value, either positive or negative, to produce desired variations of the resistance value with variations in temperature over a suitable range.

To the accomplishment of the foregoing and such other objects as will hereinafter appear, our invention consists in the elements and their relation one to the other as more particularly described hereinafter and sought to be defined in the claims; reference being had to the accompanying drawings, which show the preferred embodiment of our invention, and in which:

Figs. 1 and 2 are views showing steps of making resistance units embodying the principles of our invention, Fig. 2 showing the resistance unit in completed form.

We have found that the resistance elements or units employing painted or coated graphite films may be made with predetermined low negative or positive temperature coefficients or may be made with a substantially zero temperature coefficient by suitably combining with a film or coating of the graphite paint (possessing the negative temperature coefficient) a second film or coating of a material having a positive temperature coefficient, the two coatings being so related that the temperature coefficient of one film may be compensated or neutralized in whole or in part by the opposite temperature coefficient of the other film.

This we accomplish by constructing a resistance unit in two resistance sections having opposite temperature coefficients and by then selecting or predetermining the ratio of the resistance values of the two resistance sections in such a manner as to produce a predetermined temperature coefficient and a resulting resistance value of a desired magnitude for the composite unit. In the practice of our invention, referring now more in detail to the drawings, we first coat or paint a suitable insulating base such as 10 with a film

55

60

65

70

75

80

85

90

95

100

or layer 11 of the graphite resistance paint and we then deposit, preferably by electroplating, a second film or layer 12 of a metal such as nickel over only a portion or part of the resistance paint film 11, these layers thus forming two separate resistance sections 13 and 14. The total resistance value of the composite unit as well as the ratio of the resistance values of the sections 13 and 14 are then predetermined by arranging the resistance sections into given or selected lengths, as will be described further hereinafter.

Preferably we employ for the first film or layer 11 the paint or composition described and claimed in theforesaid patent to Lester L. Jones et al. 1,773,105, this resistance paint being composed of a finely divided graphite mixed with a binder and vehicle consisting of a metallic phosphate. In compounding the resistance material, the graphite, preferably a colloidal graphite, is mixed with a solution of aluminum in phosphoric acid to form a freely flowing paint. The aluminum in the phosphoric acid produces an aluminum phosphate; and in the preparation of the aluminum phosphate it has been found desirable to add aluminum to the phosphoric acid in such an amount as just fails to produce a precipitate. Addition of more than this amount, which would produce a precipitate, is undesirable because of the presence in the paint of large particles formed by the precipitate which interfere with the production of a smooth uniform film. On the other hand, the addition of an insufficient quantity of aluminum or aluminum phosphate is undesirable mainly because of the more highly acid condition of the resulting paint, which tends to destroy the colloidal nature of the graphite, causing clotting of the paint with streakiness in the film. It is therefore preferred to use a solution of aluminum in phosphoric acid in a slight excess of phosphoric acid, aluminum being added in such an amount as just fails to produce a precipitate. The aluminum phosphate may also be prepared by the addition of C. P. aluminum phosphate to phosphoric acid in sufficient quantity to just avoid the formation of any precipitate.

The paint thus compounded is then applied to the insulating base 10, which may be a glass or porcelain rod or a glazed or enameled surface, or may be applied to mica to form resistance coatings of very thin films of the order of magnitude of 0.1 to 0.25 thousandths of an inch, such coatings being formed in continuous and unbroken layers, as shown for example in Fig. 1 of the drawings. The paint may be applied to the insulating material by means of a brush or by dipping or by any other method. After the bases, such as 10, are coated with paint and are air-dried, the painted unit is preferably heated to ap-

proximately 500° C. for a period of approximately one hour. The heat treatment causes a reduction of the electrical resistance in the film to approximately 1% of its air-dried value. The coating or film thus formed is 70 tough and durable and may be made more or less glassy, depending upon the relative amounts of aluminum phosphate and colloidal graphite used. In lieu of colloidal graphite other forms of finely divided 75 graphite may be employed with good results, such as finely divided graphite commercially known as air floated graphite.

We have found that these graphite resistance paints or coatings may be plated 80 with a metallic coating such as 12, and that the plating may be carried out without affecting the integrity or condition of the painted coating 11. More particularly, we have discovered that with a nickel plating solution 85 the electroplating step is not critical as to the plating period nor as to the voltage or temperature of the plating bath, and that the binder of the resistance paint or film 11 is insoluble in the plating solution, these being 90 highly important advantages of the process. The plated coating 12 produced with a nickel plating solution is therefore applied over the paint coating 11 to produce the resistance section 14, the ratio of the areas of the resistance sections 13 and 14 being determined in a manner hereinafter to be described. In the electroplating step the anodes are preferably 95 symmetrically disposed with respect to the surface to be plated, this so as to obtain a 100 homogeneous deposition of the nickel. The thickness of the electrodeposit of the nickel film is preferably of the same order of magnitude as that of the paint film, and is about 0.2 thousandths of an inch. The plating solution 105 is substantially neutral to the paint film 11 and hence the paint film is unattacked, and we have found it unnecessary to treat the units to remove traces of any chemicals of the plating bath. Moreover, the paint film 11 110 which adheres very firmly to the insulating base 10 forms a firm basis or support for the deposited or plated metal film. Fig. 1 of the drawings shows the embryo resistance element produced by the steps thus far described, the thicknesses of the films being 115 exaggerated for purposes of elucidation.

To predetermine the temperature coefficient for the resistance element, the resistance values of the sections 13 and 14 of 120 the unit are predetermined so as to have a given ratio and a desired additive or resulting resistance. To permit of a uniform heat dissipation over both sections of the unit, the respective areas of the sections are also given 125 a selected ratio. We have found that the best results are achieved by making the ratio of the resistance values of the two sections equal to the inverse ratio of the temperature coefficients of the films taken over the range 130

of temperatures in which the units are to be used. Thus with a range of temperature variation between room temperature and 160° C. the negative temperature coefficient 5 of the paint film 11 is about 15%, while the positive temperature coefficient of the plated film 12 is about 50%. The resistance values of the sections 14 and 13 are therefore selected to have a ratio of 15 to 50. The areas of the 10 sections 13 and 14 are preferably determined by the resistance values of the sections at the average operating temperature thereof. Thus the areas are given the same ratio as the resistance values of the sections at say an 15 operating temperature of 160° C. In the example stated, the areas of the sections 14 and 13 will have a ratio of about 7 to 13. The unit thus constructed is designed for complete 20 neutralization of the negative temperature coefficient by the positive temperature coefficient; and it is found that the unit is non-critical in that the same may be operated within a range of 140° to 180° C. with only small deviations from zero temperature 25 coefficient, the deviations over the entire range from room temperature to 160° C. being of the order of 1%.

The preferred way of imparting the desired resistance values to the resistance sections 30 14 and 13 to obtain the desired resistance ratio and resultant is by employing the spiralling method disclosed and claimed in the patent to Lester L. Jones, No. 1,635,184 of July 12, 1927. In accordance with this method, the insulating base is made in cylindrical 35 form and the resistance layer thereon is provided with a helical groove cut along the base, the helix being cut to a length for producing a resistance of a given or desired value. Applying 40 this method, both the sections 14 and 13 are cut helically, preferably in a lathe, so as to provide the helical strip 16 for the section 14 and the helical strip 17 for the resistance section 13, as shown in Fig. 2 of the drawings. Due to the fact that the specific 45 conductance of the resistance layer 12 is much greater than that of the paint film 11, the pitch of the helix strip 16 is much smaller than that of the helix strip 17, all as depicted 50 in Fig. 2 of the drawings. It will be understood that in cutting the helical grooves the resistance values of the two sections of the element are first determined and then obtained after the manner disclosed in said Patent 55 No. 1,635,184.

If the resistance units are made on enameled iron or enameled brass or copper, the ratio of areas need not be selected as hereinbefore set forth, since the heat conduction 60 through the metal base tends to equalize the temperatures of the nickel and paint sections. The aforesaid desired ratio of resistance areas is therefore preferred only when the heat dissipation is by radiation or convection. Slight variations in the area ratio

serve to change the temperature at which the total resistance is exactly the same as the initial resistance (at room temperature). The completed resistance element is provided with contact terminals in the form of metallic bands 18 and 19 which are clamped over the ends of the paint resistance film 11, as shown in Fig. 2 of the drawings. 70

The arithmetic example heretofore given for the resistance ratios and ratio of resistance areas is for a resistance unit having a zero temperature coefficient. It will be understood that a variation from this resistance ratio on one side or the other will produce either a predetermined negative or a predetermined positive temperature coefficient for the unit. The principles of the invention may therefore be employed in producing resistance elements having small and intended values of resistance variations with temperature either in a positive direction or in a negative direction. 75 80 85

The manner of making and using resistance units embodying our invention and the many advantages thereof will in the main be fully apparent from the above detailed description thereof. It will be further apparent that while we have shown and described our invention in the preferred form, many changes and modifications may be made in 90 the structure disclosed without departing from the spirit of the invention, defined in the following claims. 95

We claim:

1. The method of manufacturing a non-hygroscopic high resistance unit having a desired temperature coefficient, which includes coating the surface of an insulation base with a high resistance coating comprising colloidal graphite suspended in a vehicle including a metallic phosphate in an excess of phosphoric acid, baking the resulting unit to form a high resistance film having a negative temperature coefficient, and coating a portion of the graphite surface with a thin film of metallic nickel in order to form a resistance film having a positive temperature coefficient, the graphite and nickel resistance films being relatively proportioned to obtain the desired over-all temperature coefficient, and being further proportioned to obtain an over-all series resistance equal to the desired resistance of the unit. 100 105 110 115

2. The method of manufacturing a non-hygroscopic high resistance unit having a zero temperature coefficient, which includes coating the surface of an insulation base with a high resistance coating comprising finely divided graphite suspended in a vehicle including a metallic phosphate, baking the resulting unit to form a high resistance film having a negative temperature coefficient, and coating a portion of the graphite surface with a thin film of metal in order to form a resistance film having a positive temperature 120 125 130

coefficient, the graphite and metal resistance films being proportioned to obtain graphite and metal resistance values inversely proportional to the respective temperature coefficients at a predetermined operating temperature, and an over-all series resistance equal to the desired resistance of the unit.

3. The method of manufacturing a non-hygroscopic high resistance unit having a zero temperature coefficient, which includes coating the surface of an insulation base with a high resistance coating comprising finely divided graphite suspended in a vehicle including a metallic phosphate and baking the resulting unit to form a high resistance film having a negative temperature coefficient, coating a portion of the graphite surface with a thin film of metal in order to form a resistance film having a positive temperature coefficient, and thereafter appropriately cutting the graphite and metal resistance films to obtain graphite and metal resistance values inversely proportional to the respective temperature coefficients at a predetermined operating temperature, and an over-all series resistance equal to the desired resistance of the unit.

4. The method of manufacturing a non-hygroscopic high resistance unit having a zero temperature coefficient, which includes coating the entire external surface of a cylindrical insulation base with a high resistance coating comprising colloidal graphite suspended in a vehicle including a metallic phosphate in an excess of phosphoric acid and baking the resulting unit to form a high resistance film having a negative temperature coefficient, electro-plating a portion of the coated surface with a thin film of metallic nickel in order to form a resistance film having a positive temperature coefficient, and thereafter spiral cutting the graphite and nickel resistance films at pitches appropriate to obtain graphite and nickel resistance values inversely proportional to the respective temperature coefficients at a predetermined operating temperature, and an over-all series resistance equal to the desired resistance of the unit.

5. The method of manufacturing a non-hygroscopic high resistance unit having a zero temperature coefficient, which includes coating the surface of an insulation base with a high resistance coating comprising colloidal graphite suspended in a vehicle including a metallic phosphate in an excess of phosphoric acid and baking the resulting unit to form a high resistance film having a negative temperature coefficient, and plating a portion of the coated surface with a thin film of metallic nickel in order to form a resistance film having a positive temperature coefficient, the areas of the plated and unplated portions of the resistance unit being proportional to the desired respective resistance values, the

resistance values being inversely proportional to the respective temperature coefficients at a predetermined operating temperature, and the over-all series resistance being equal to the desired resistance of the unit.

6. A non-hygroscopic high resistance unit having a desired temperature coefficient comprising an insulation base the surface of which is coated with a thin film of colloidal graphite held in a binding metallic phosphate vehicle and forming a high resistance film having a negative temperature coefficient, and a thin film of metallic nickel plated over only a portion of the resulting graphite film in order to form a resistance film having a positive temperature coefficient, the resulting resistance films being properly relatively proportioned to obtain the desired over-all temperature coefficient, and being further proportioned to obtain an over-all series resistance equal to the desired resistance for the unit.

7. A non-hygroscopic high resistance unit having a zero temperature coefficient comprising an insulation base the surface of which is coated with a thin film of finely divided graphite held in a binding metallic phosphate vehicle and forming a high resistance film having a negative temperature coefficient, and a thin film of metal coated over only a portion of the resulting graphite film in order to form a resistance film having a positive temperature coefficient, the resulting resistance films being properly proportioned to obtain resistance values inversely proportional to the temperature coefficients at a predetermined operating temperature, and an over-all series resistance equal to the desired resistance for the unit.

8. A non-hygroscopic high resistance unit having a zero temperature coefficient comprising an insulation base the external surface of which is coated with a thin film of finely divided graphite held in a binding metallic phosphate vehicle and forming a high resistance film having a negative temperature coefficient, and a thin film of metal coated over only a portion of the resulting graphite film in order to form a resistance film having a positive temperature coefficient, the resulting resistance films being cut to obtain resistance values inversely proportional to the temperature coefficients at a predetermined operating temperature, and an over-all series resistance equal to the desired resistance for the unit.

9. A non-hygroscopic high resistance unit having a zero temperature coefficient comprising a cylindrical insulation base the external surface of which is coated with a thin film of colloidal graphite held in a binding metallic phosphate vehicle and forming a high resistance film having a negative temperature coefficient, and a thin film of metallic nickel plated over only a portion of the

resulting graphite film in order to form a resistance film having a positive temperature coefficient, the resulting resistance films being spirally cut at pitches properly selected to obtain resistance values inversely proportional to the temperature coefficients at a predetermined operating temperature, and an over-all series resistance equal to the desired resistance for the unit.

10 10. A non-hygrosopic high resistance unit having a zero temperature coefficient comprising an insulation base the surface of which is coated with a thin film of colloidal graphite held in a binding metallic phosphate vehicle and forming a high resistance film having a negative temperature coefficient, a thin film of metallic nickel plated over only a portion of the resulting graphite film in order to form a resistance film having a positive temperature coefficient, the areas of the plated and unplated portions of the resistance unit being proportional to the respective desired resistance values, the resistance values being inversely proportional to the temperature coefficients at a predetermined operating temperature, and the over-all series resistance being equal to the desired resistance for the unit.

20 Signed at New York in the county of New York and State of New York this 5th day of March A. D. 1928.

25 LESTER L. JONES.  
JOSEPH A. FLANZER.

35

40

45

50

55

60